

## 1

3,035,906

SYNERGISTIC ADDITIVE MIXTURES FOR FUELS  
James B. Hinkamp, Birmingham, Mich., assignor to Ethyl Corporation, New York, N.Y., a corporation of Delaware  
No Drawing. Filed May 28, 1958, Ser. No. 738,284  
6 Claims. (Cl. 44—66)

New non-corrosive gasoline additives having strong anti-icing properties are among the objects of this invention.

The additives are the  $\beta$ -hydroxyethyl ethylenediamine amides of oleic acid (henceforth MPA) mixed with methyl phosphates. As little as 0.5 percent by weight of MPA makes the mixtures non-corrosive to ferrous metals when water is present and even when storage temperatures are high (90–120° F.). Absent MPA, the phosphates corrode ferrous metals under these conditions.

Because MPA itself is non-corrosive, there is no necessary upper limit on the amount used with the phosphates. Costwise, up to about 75 percent of MPA in the mixture is very good.

The methyl phosphates have the formula



$\text{R}_1$  and  $\text{R}_2$  being methyl, phenyl, tolyl or xylyl. Of these compounds trimethyl phosphate is most easily hydrolyzed. Therefore, when water seeps or otherwise gets into iron drums or cans in which it is stored, there is drastic corrosion. Yet strangely, this does not happen when MPA is present. Instead, metal corrosion is sharply reduced.

Much harder to hydrolyze are the other above phosphates—e.g., dimethyl xylyl phosphate, methyl ditolyl phosphate, etc. But to the extent they do hydrolyze under rough treatment, there is a commercial problem. Certain mixtures of these phosphates are commercially-used ignition control compounds for motor fuel and their metal shipping drums are often exposed to rain, high temperatures, etc. Result if the water gets inside: Hydrolysis of the phosphate and consequent corrosion. But joint use of MPA squelches and problem.

Also non-corrosive are hydrocarbon solutions of these MPA-phosphate mixes. For instance, gasoline stock or blending solutions of high phosphate content (e.g., 10–20 weight percent) containing MPA (0.5 weight percent or more based on the phosphate) do not corrode iron or steel tanks, pipelines, etc., though water be present and temperatures high. More dilute gasoline solutions are likewise non-corrosive even when stored for years over water.

Another big feature of gasoline-phosphate-MPA systems is their potent anti-icing properties. They quash the frequent stalling of automotive, marine, stationary and airplane engines normally suffered during running—mostly at idle—in cool, moist weather. This feature exists in gasoline containing (by weight) about 75–550 parts per million (p.p.m.) of the above phosphates and about 15–200 p.p.m. of MPA, the total phosphate-MPA content being at least 130 p.p.m.

Synergistic anti-icing effects exist in the above fuels with MPA and the phosphates which have up to 2 methyl ester groups—dimethyl phenyl, dimethyl tolyl, dimethyl xylyl, methyl diphenyl, methyl ditolyl, and methyl dixylyl phosphates. Mixtures of these phosphates are likewise synergistic with MPA. A preferred synergistic fuel of this invention is gasoline containing about 15–100 p.p.m. of MPA and about 200–450 p.p.m. of the phosphates having up to 2 methyl ester groups, especially a mixture composed predominantly of dimethyl xylyl phosphate and

## 2

methyl dixylyl phosphate, about four-fifths of the phosphate mixture being the dimethyl compound.

These anti-corrosion and anti-stalling properties persist in the presence or absence of other fuel additives. Thus, the fuel may be leaded. It may contain other antiknock—e.g., methylcyclopentadienyl manganese tricarbonyl, etc. Antioxidants, metal deactivators, dyes, aromatic solvents (e.g., xylene, etc.) and the like may be present. In every case, the benefits of this invention are fully realized.

- 10 On top of all this, my MPA-phosphate mixtures cause no problems in use. They are liquids that are easy to blend with fuel even in the cold. They do not harm fuel stability. They are perfectly engine-inductible. And they form no harmful engine deposits.
- 15 MPA and some of the phosphates are now being sold. MPA is made by heating oleic acid with  $\beta$ -hydroxyethyl ethylenediamine under azeotropic conditions to form the imidazoline



20 This is then treated with water to form MPA, i.e., a mixture of the amides



30 and



- 35 It is best to mix these amides with 30–40 percent aromatics of the xylene range, 3–8 percent butanol (lowers freezing point) and about 4 percent water (prevents jelling in the cold and keeps the imidazoline hydrolyzed). When so formulated, MPA is an amber liquid. Typical 40 properties: gravity, ° API (ASTM D-287) 20–25; pour point, ° F. (ASTM D-97), ca. 15; viscosity at 100° F., SSU (ASTM D-445 and 446), ca. 260; total base number, mg. KOH/gram 75–85.

The phosphates can be made by reacting  $\text{POCl}_3$  with 45 the right amount of phenol, cresol, xylol and/or methanol.  $\text{HCl}$  is given off and the ester formed. Details for making trimethyl phosphate are well known and described in the literature. The dimethyl aryl phosphates are best made by first reacting (mole per mole) the 50 phenol in question with  $\text{POCl}_3$ . Use is made of  $\text{AlCl}_3$  as catalyst—0.25–3.0 mole percent based on the phenol. Temperature: 85–130° C. The phenol should be fed a little at a time to the  $\text{POCl}_3$ . The product—a phenyl phosphorodichloride—is then added slowly to methanol 55 (at least 4 moles per mole of  $\text{POCl}_3$  first used). Keep the mixture at 15–60° C. until all the product is added. Then, quench with water and distill off the ester from the organic phase at reduced pressure (dimethyl phenyl phosphate 114° C. at 2 mm.; dimethyl tolyl phosphate 113–115° C. at 1 mm.; dimethyl xylyl phosphate 113–115° C. at 0.5 mm.). The methyl diaryl phosphates are 60 made the same way except that the ratios are changed (phenol:  $\text{POCl}_3$  is 2:1 and at least two moles of methanol are used per mole of  $\text{POCl}_3$ ). The end products distill at slightly higher temperatures than the dimethyl aryl phosphates. All of these phosphates are clear white or light yellow liquids.

To make my MPA-phosphate mixtures, apt amounts of each are blended in a tank, can or other vessel. A little stirring or shaking helps. No special precautions need be taken.

70 My fuels can be made by blending the correct amount

of one of my MPA-phosphate blends with the gasoline. If desired, a fuel concentrate can first be made for use in later fuel blending steps. Then again my fuels can be made by blending first one and then the other of my additives with the gasoline. As before, the correct amount of each can be used in the first instance or a fuel concentrate can be formed and cut with more gasoline to the desired level. Other additives, if used, can be blended before, during or after the above fuel blending steps.

In the examples below, parts and percents are by weight.

#### EXAMPLE I

Mixed are 99.5 parts of methyl dixylyl phosphate and 0.5 parts (0.5 percent) of MPA. The liquid is non-corrosive to ferrous metals when placed in contact with water.

#### EXAMPLE II

To 75 parts of MPA is added 25 parts of dimethyl phenyl phosphate. They are mixed. The liquid composed of 75 percent MPA is not corrosive to strips of iron when resting on a water layer and held at 120° F. for days on end.

#### EXAMPLE III

Mixed are 90 parts of trimethyl phosphate and 10 parts (10 percent) of MPA. The liquid product is much less corrosive of steel drums when water is present than is the pure phosphate.

#### EXAMPLE IV

A 50 percent MPA-methyl ditolyl phosphate mixture—made from 50 parts of each—and also 10 and 20 percent gasoline solutions of this mixture are found non-corrosive to ferrous metals in the presence of water.

#### EXAMPLE V

Stirred with 990 parts of mixed methyl tolyl phosphates ( $d_4^{20}$  1.113;  $n_D^{20}$  1.496) is 10 parts of MPA (1 percent). The liquid product is non-corrosive to iron drums in which water has gathered.

#### EXAMPLE VI

Mixed are 500 parts of dimethyl xyllyl phosphate and 15 parts (2.9 percent) of MPA. This mixture is blended with  $10^6$  parts of motor fuel. It contains 500 p.p.m. of the phosphate and 15 p.p.m. of MPA. The fuel is non-corrosive to storage tanks. It has strong anti-stalling properties in use.

#### EXAMPLE VII

With  $10^6$  parts of aviation fuel containing 4.6 ml./gal. of tetraethyllead (TEL) as 1-T Mix is added 200 parts (200 p.p.m.) of MPA. Next is added 75 parts (75 p.p.m.) of trimethyl phosphate. The mixture is stirred. The finished fuel is non-corrosive to ferrous metals and has good de-icer quality. NOTE.—1-T Mix is made up mostly of TEL and 1 theory of ethylene dibromide. A theory is 2 halide atoms per lead atom.

Other examples vis-a-vis engine test work are given below.

The test set up was a 1953 car engine drawing its air from outdoors through an ice tower. The carburetor had a water-jacketed throttle body through which ice water was passed to keep the throttle blade cold. The intake air temperature was controlled by blending inside air with the outside air at the entrance to the ice tower. All tests were run when outside temperatures were below 40° F. In this way, icing and stalling were obtained in short times. Test details:

(1) Engine run at 1500 r.p.m. idle until reached—

Intake air: 38 to 40° F. (dry bulb)

36° +

Throttle blade: 20 to 25° F.

Jacket water out: 135 to 140° F.

Oil sump: 165-175° F.

- (2) Flushed fuel system with a non-icing fuel.
- (3) Switched to test fuel and ran at 1500 r.p.m. idle for two minutes.
- (4) Set engine to 450-500 r.p.m. idle and without further throttle changes, observed time to stall.

All test fuels contained 3.0 ml. TEL/gal. as 62-Mix. This is chiefly TEL, 0.5 theory of ethylene dibromide and 1.0 theory of ethylene dichloride.

In the table are the test results:

Table.—Effect of Additives on Engine Stalling

| No. | Additive                             | Cone., p.p.m. | Average Increase in Stall Time, Percent |
|-----|--------------------------------------|---------------|-----------------------------------------|
| 1   | Methyl xyllyl phosphate <sup>1</sup> | 220           | 13                                      |
| 2   | do                                   | 440           | 57                                      |
| 3   | MPA                                  | 50            | 47                                      |
| 4   | MPA                                  | 100           | 83                                      |
| 5   | Methyl xyllyl phosphate + MPA        | 440: 50       | 246                                     |
| 6   | do                                   | 220: 15       | 97                                      |

<sup>1</sup> Dimethyl xyllyl phosphate: methyl dixylyl phosphate ca. 80:20 wt. percent.

Note from items 5 and 6 that my fuels were synergistic. By the same test method, 1.5 volume percent of isopropanol—a widely used deicer—gave only a 45 percent increase in stall time. This further shows the great anti-stalling strength of my fuels.

I claim:

1. A fuel additive composition consisting essentially of a phosphate having the formula



wherein  $R_1$  and  $R_2$  are selected from the group consisting of methyl, phenyl, tolyl and xyllyl, and the  $\beta$ -hydroxyethyl ethylenediamine amides of oleic acid; said additive containing from 0.5 to 75 percent by weight of said amides.

2. Gasoline containing by weight about 75-550 parts per million of a phosphate having the formula



wherein  $R_1$  and  $R_2$  are selected from the group consisting of methyl, phenyl, tolyl and xyllyl, and about 15-200 parts per million of the  $\beta$ -hydroxyethyl ethylenediamine amides of oleic acid, the total content of said phosphate and amides being at least 130 parts per million.

3. Gasoline containing by weight about 200-450 parts per million of a phosphate having the formula



wherein  $R_1$  and  $R_2$  are selected from the group consisting of methyl, phenyl, tolyl and xyllyl, and about 15-100 parts per million of the  $\beta$ -hydroxyethyl ethylenediamine amides of oleic acid.

4. The gasoline composition of claim 2 wherein said phosphate has up to 2 methyl ester groups.

5. The gasoline composition of claim 3 wherein said phosphate has up to 2 methyl ester groups.

6. Gasoline containing by weight from about 220 to about 440 parts per million of a mixture comprising about 80 percent by weight of dimethyl xyllyl phosphate and approximately 20 percent by weight of methyl dixylyl

phosphate, and about 15 to 50 parts per million of the  $\beta$ -hydroxyethyl ethylenediamine amides of oleic acid.

**References Cited** in the file of this patent

UNITED STATES PATENTS

|           |                      |               |
|-----------|----------------------|---------------|
| 2,080,299 | Benning et al. ----- | May 11, 1937  |
| 2,089,212 | Kritchevsky -----    | Aug. 10, 1937 |
| 2,167,867 | Benning -----        | Aug. 1, 1939  |

5 2,604,451  
2,839,373  
2,843,464

2,851,343  
2,856,299  
2,862,800

600,191

|                       |               |
|-----------------------|---------------|
| Rocchini -----        | July 22, 1952 |
| Barusch et al. -----  | June 17, 1958 |
| Gaston -----          | July 15, 1958 |
| Cantrell et al. ----- | Sept. 9, 1958 |
| Westlund -----        | Oct. 14, 1958 |
| Cantrell et al. ----- | Dec. 2, 1958  |

FOREIGN PATENTS

|                     |              |
|---------------------|--------------|
| Great Britain ----- | Apr. 2, 1948 |
|---------------------|--------------|

UNITED STATES PATENT OFFICE  
CERTIFICATE OF CORRECTION

Patent No. 3,035,906

May 22, 1962

James B. Hinkamp

It is hereby certified that error appears in the above numbered patent requiring correction and that the said Letters Patent should read as corrected below.

Column 2, lines 19 to 24, the formula should appear as shown below instead of as in the patent:



Signed and sealed this 4th day of September 1962.

(SEAL)

Attest:

ERNEST W. SWIDER

Attesting Officer

DAVID L. LADD

Commissioner of Patents